

H. H. ROBERTSON.  
PROTECTED METAL ARTICLE AND PROCESS OF MAKING SAME.  
APPLICATION FILED JUNE 3, 1916.

1,195,090.

Patented Aug. 15, 1916.

*Fig. 1.*



*Fig. 2.*



*Inventor*  
Harold H. Robertson  
by Jas. H. Lunnell  
Atq.

# UNITED STATES PATENT OFFICE.

HAROLD H. ROBERTSON, OF SEWICKLEY, PENNSYLVANIA, ASSIGNOR TO ASBESTOS PROTECTED METAL COMPANY, OF PITTSBURGH, PENNSYLVANIA, A CORPORATION OF PENNSYLVANIA.

## PROTECTED METAL ARTICLE AND PROCESS OF MAKING SAME.

1,195,090.

Specification of Letters Patent. Patented Aug. 15, 1916.

Application filed June 3, 1916. Serial No. 101,635.

To all whom it may concern:

Be it known that I, HAROLD H. ROBERTSON, a subject of the King of Great Britain, and a resident of Sewickley, in the county of Allegheny and State of Pennsylvania, have invented an Improvement in Protected Metal Articles and Processes of Making Same, of which the following description, in connection with the accompanying drawings, is a specification, like characters on the drawings representing like parts.

This invention relates to a protected metal article and to the process of making the same, and particularly to a metal article having a covering or layer of fibrous material adhesively secured to the metal article by asphalt or like cementitious material.

The present invention has for its object to produce a metal article, such as an iron or steel sheet or layer with a protective coating of asphalt or other cementitious material, which is united with the metal sheet or layer in a superior manner. To this end the metal sheet or article after being cleaned as by picking, etc., as now commonly practised in cleaning metal sheets, is provided with a coating or layer of a material capable of resisting a relatively high temperature, which material will be hereinafter referred to as a lacquer, and the lacquered metal sheet is then dried by subjecting it to heat to set or bake the coating, after which it is passed through a bath of protective material, such as asphalt, which does not have a detrimental effect on the coating of lacquer but unites therewith to effectively secure the asphalt layer to the metal article. The metal article thus protected may be further protected by layers of fibrous material, such as asbestos, felt and the like, which may be saturated with asphalt or like material, or which may not be saturated, and which may be given a surface coating or layer to incase the fibrous material within it. These and other features of this invention will be pointed out in the claims at the end of this specification.

Figure 1 is a plan view with parts broken away of a protected metal sheet embodying the invention, and Fig. 2, a section on the line 2—2, Fig. 1.

Referring to Fig. 1, *a* represents a metal sheet, preferably of iron or steel, which is provided on its opposite surfaces and edges

with a coating or layer *b* of lacquer capable of resisting a relatively high temperature. The metal sheet *a* provided with the coating or layer *b* of lacquer is subjected to heat to dry and set the lacquer, and is then passed through a bath of asphalt or like cementitious material to provide the metal sheet with a coating or layer *c* of asphalt or the like, which adheres firmly to the layer *b* of lacquer and is thereby firmly secured to the metal sheet *a*.

It is preferred to use as the foundation coating a lacquer which is more or less resistant to acids and alkalis, proof against moisture, flexible, and capable of resisting a relatively high temperature.

I have found that a lacquer composed of a vegetable oil, a thinning material and a bituminous or coal tar product, such, for instance, as linseed oil, benzol and Gilsonite or a coal tar resin, vegetable oil and turpentine, is suitable for my purpose, and while it may be preferred to use either of the particular lacquers described, it is not desired to limit the invention in this respect, as any lacquer having the characteristics above noted, may be used.

A metal sheet protected as above described, may be used without further protection; but for certain purposes, as, for instance, when used as the roofing and siding of buildings, it is preferred to provide additional protection, and for this purpose the protected metal sheet may have secured to it layers *d* of asbestos, paper, felt or other fibrous material, which may be saturated with asphalt of a relatively low melting point, marked *e* in Fig. 1, or which may not be saturated but left in their natural condition.

The non-saturated fibrous layers *d* are adhesively secured to the metal sheet *a* by the layer *c* of asphalt and the saturated layers by the layer *c* assisted by the saturating asphalt *e*, which unites with the layer *c*. When the asbestos or other fibrous layers *d* are saturated with asphalt or the like of relatively low melting point, the metal sheet may be further protected by a surface layer *f* of asphalt having a relatively high melting point, which unites with the saturating material of the fibrous layers and seals the volatile constituents of the saturating material, thereby retaining the latter in its

effective condition to protect the primary asphalt layer and the lacquer from the detrimental action of climatic changes, fumes, gases, etc., and also as an enveloping binder for the fibrous layers, and, as a result, the metal sheet is thoroughly protected against extraneous influences for a substantially long time. A lacquer capable of resisting a substantially high temperature, is especially advantageous as it is capable of being baked or heated in a suitable oven in a substantially short time and permits the lacquered sheets to be stacked or piled up without danger of sticking to one another, and further is capable of being passed through a bath of asphalt, and effectively unites the asphalt to the iron or steel sheet or other metal article, inasmuch as the adhesion of the lacquer to the metal is superior to that of the asphalt to the metal, and the adhesion of the asphalt to the lacquer is superior to that of the asphalt to the metal, and further the lacquer is also a resistant to acid and alkali fumes and gases and to moisture and is of increased flexibility, which latter allows the metal sheet to be bent more or less without exposing the metal. In other words, a superior protection for the metal sheet against corrosion is obtained by means of the coatings or layers of lacquer and asphalt, and a superior adhesion of the asphalt with the metal sheet is obtained, consequently when the said sheet is provided with protective layers of asbestos, felt or paper and like fibrous material, a superior bonding or adhesion of the fibrous layers to the metal sheet or article is obtained, with the result that a more durable and commercial article is produced.

40 I claim:

1. An improved article of manufacture comprising a metal article provided with a coating of lacquer applied to the metal article, and a coating or layer of asphalt applied to the coating of lacquer.
2. An improved article of manufacture, comprising a metal article provided with a coating of lacquer capable of resisting a relatively high temperature, and a coating of asphalt applied to the coating of lacquer.

3. An improved article of manufacture comprising a metal article provided with a coating of lacquer applied to the metal article, a coating or layer of asphalt applied to the coating of lacquer, and a protective layer of fibrous material affixed to the said asphalt coating.

4. An improved article of manufacture comprising a metal article provided with a coating of lacquer applied to the metal article, a coating or layer of asphalt applied to the coating of lacquer, and a protective layer of fibrous material saturated with asphalt and affixed to said asphalt coating.

5. An improved article of manufacture comprising a metal article provided with a coating of lacquer applied to the metal article, a coating or layer of asphalt applied to the coating of lacquer, a protective layer of fibrous material saturated with asphalt and affixed to said asphalt coating, and a surface coating applied to the external surface of the saturated fibrous layers to seal the volatile constituents of the saturating material of said fibrous layers and to bind the fibrous layers to the metal article.

6. The method of protecting metal articles, which consists in cleaning the same, applying to the cleaned metal article a coating of lacquer, subjecting the lacquered article to heat to dry the same, and applying to the lacquered article a coating of asphalt.

7. The method of protecting metal articles, which consists in cleaning the same, applying to the cleaned metal article a coating of lacquer, subjecting the lacquered article to heat to dry the same, and passing the lacquered article through a bath of asphalt.

8. The method of protecting metal articles, which consists in cleaning the same, applying to the cleaned metal article a coating of lacquer, subjecting the lacquered article to heat to dry the same, passing the lacquered article through a bath of asphalt and applying a fibrous material to the asphalt coated article.

In testimony whereof, I have signed my name to this specification.

HAROLD H. ROBERTSON.

It is hereby certified that in Letters Patent No. 1,195,090, granted August 15, 1916, upon the application of Harold H. Robertson, of Sewickley, Pennsylvania, for an improvement in "Protected Metal Articles and Processes of Making Same," an error appears in the printed specification requiring correction as follows: Page 1, line 25, for the word "picking" read *pickling*; and that the said Letters Patent should be read with this correction therein that the same may conform to the record of the case in the Patent Office.

Signed and sealed this 24th day of October, A. D., 1916.

[SEAL.]

F. W. H. CLAY,

*Acting Commissioner of Patents.*